

## UNITED STATES PATENT OFFICE

2,436,219

## TEXTILE PRODUCT AND PROCESS

Robert D. MacLaurin, Lakewood, Ohio, assignor  
to Industrial Rayon Corporation, Cleveland,  
Ohio, a corporation of Delaware

No Drawing. Application November 1, 1944,  
Serial No. 561,498

12 Claims. (Cl. 252—8.9)

1

This invention relates to the production of improved filaments, yarns, threads and the like which have been treated with improved yarn-treating and conditioning compositions. This invention also provides new and improved yarn-conditioning compositions. For the purposes herein, the term "yarn" is meant to include filaments, threads, and the like used in the production of textiles.

In the knitting and weaving of textile products it is common practice to use textile yarns which have been subjected to a desired amount of twisting. In performing the twisting operations and in the weaving and knitting steps themselves, it is necessary to pass the yarns over a variety of guides, bobbins and other mechanical devices which offer frictional resistance to the yarn and which, accordingly, tend to subject the yarn to abrasive action. It is of course desirable to eliminate such abrasive wear as completely as possible.

This invention provides a new yarn-treating and conditioning composition which makes possible the production of yarns which offer a very substantially reduced frictional resistance to the various mechanical devices over which the yarn travels in the course of twisting, knitting or weaving operations with the result that abrasive wear is kept to a minimum. In addition, yarn which has been treated with the new compositions of this invention has its twist somewhat stabilized or set so that the yarn has less tendency to snarl or become knotted in passing over the various yarn guides, etc., incident to its formation into knitted or woven products. A further advantage of yarns which have been treated with the new compositions is that the filaments comprising the yarn are protected by the new conditioning composition so that they are less apt to snag during the course of the knitting or weaving operation. The new yarns of this invention may be used with particular advantage in the production of hosiery.

An important advantage of the new yarn-conditioning compositions is that they may be readily removed from the yarn after the yarn has been knitted or woven into a textile product. The yarn-conditioning composition may be readily and effectively removed by means of ordinary aqueous washing or detergent compositions. A further advantage of the new yarn-conditioning compositions is that the coefficient of friction of the yarn to which the composition is applied is not so low as to permit excessive slippage of the yarn during its manufacture into a textile product and, consequently, non-uniformity of the fabric due to this cause is minimized.

The new yarn-conditioning composition is not corrosive to the various parts of the textile fabricating devices with which the yarn comes into contact and, in addition, the composition does not

2

tend to clog yarn guides, knitting needles, etc. The new yarn-conditioning composition is chemically and physically stable both in storage and after application to the yarn.

5 The new yarn-conditioning composition comprises a hydrogenated fish oil and a product formed by reacting an alkylene oxide with a partial polyester of a fatty acid containing at least 12 carbon atoms and a polyhydric alcohol such as the hexahydric alcohols and their anhydro derivatives. New yarn products are produced in accordance with this invention by treating yarn with this yarn-conditioning composition.

10 The hydrogenated fish oils employed in practicing this invention are solid and waxy in nature and advantageously have iodine numbers below 50 and a melting point between about 30° C. and 60° C. and particularly having an iodine number below 45 and a melting point between about 40° C. and 55° C.

15 The alkylene oxide reaction products employed in the yarn-conditioning composition of this invention may be prepared by known methods of reacting an alkylene oxide with a partial fatty acid polyester under elevated pressures in the presence of suitable catalysts such as, for example, alkali metal hydroxides, e. g., sodium and potassium hydroxide, and alkali metal alkoxides such as sodium methoxide, etc. Alkylene oxide reaction 20 products which may be used with advantage are those prepared by reacting at least about 20 moles of the alkylene oxide with one mole of the ester. The alkylene oxides employed may include compounds such as ethylene oxide and propylene oxide although the employment of ethylene oxide is preferred.

25 The partial fatty acid polyester may be derived from such hexahydric alcohols and their anhydro derivatives as sorbitol, mannitol, dulcitol, sorbitan and mannitan. The fatty acid portion of the ester is advantageously derived from fatty acids containing at least 12 carbon atoms and may include saturated fatty acids such as lauric, myristic, palmitic and stearic, and unsaturated 30 and hydroxy fatty acids such as oleic, ricinoleic, etc. The partial polyesters may advantageously be either predominantly di-esters, tri-esters or mixtures thereof. The partial polyesters all contain unesterified portions of the alcoholic residue of the ester which are capable of being reacted with an alkylene oxide.

35 Among the specific partial polyesters which may be reacted with at least about 20 moles of an alkylene oxide, e. g., ethylene oxide, to produce one of the components of the new yarn-conditioning composition may be mentioned sorbitan trioleate, mannitan trioleate, sorbitan trilaurate, mannitan trilaurate, etc.

40 In making up the yarn-treating composition of this invention, the proportions, by weight, may

advantageously be about 0.82 to 1 parts of hydrogenated fish oil to about 1 part of the alkylene oxide reaction product. These components of the composition may advantageously be mixed or blended by heating them until a molten mass is obtained. The presence of small amounts of water, e. g., from 5 to 10%, in the alkylene oxide reaction product facilitates admixture and blending of this component with the hydrogenated fish oil.

Although the composition may be applied to yarn in the molten or undiluted form, it is more advantageously applied in a diluted form, such as a solution or dispersion, depending somewhat upon the degree of solubility or dispersibility of the composition in the medium employed. It is particularly advantageous to apply the composition in the form of solutions or dispersions containing about 3% to 5.0%, by weight in the aggregate, of the hydrogenated fish oil and the alkylene oxide reaction product. In making up aqueous dispersions, it is advantageous to use up to about 0.5% (based on the aggregate weight of the hydrogenated fish oil and alkylene oxide reaction product) of a suitable alkaline dispersing agent such as an alkylolamine, e. g., triethanolamine. Small amounts of tetrachlorphenol may also be added to the dispersion as a stabilizer.

It has been found to be particularly advantageous to use aqueous dispersions in which the dispersed particles are of extremely small size, for example, dispersions having light transmissions of at least about 80% by the Fischer Electrophotometer A. C. Model at 1.5%, by weight, concentrations, and when containing only the hydrogenated fish oil and alkylene oxide reaction products of the yarn-conditioning composition of this invention.

The composition of this invention is advantageously applied to the yarn prior to the twisting operations. The treated yarn may, if desired, be dried before being subjected to twisting. In the production of textile materials from yarns such as regenerated cellulosic yarns, it is particularly advantageous to treat the yarn before it has been subjected to the first drying stage normally incident to its production. This may be done with especial advantage when viscose rayon, for example, is produced by the continuous process as described in Torrence Patent No. 2,284,497 by applying an aqueous dispersion of the yarn-treating composition to the viscose rayon just prior to the delivery of the yarn to the drying reel on which the yarn is continuously dried prior to twisting. The amount of the composition deposited on the yarn may range from about .75 to 10%, by weight, of the yarn and more advantageously from 2% to about 4%. The invention will be more fully described by reference to the following example although it is to be understood that the invention is not limited thereto.

#### Example

47 pounds of a hydrogenated fish oil was added to 50.25 pounds of a product produced by reacting about 20 moles of ethylene oxide with one mole of sorbitan trioleate. The hydrogenated fish oil had a melting point of about 50° C., an iodine number of about 30, less than 0.5% free fatty acid and a saponification number of about 190. The ethylene oxide reaction product is a syrupy liquid containing about 5% water and having a specific gravity at 25° C. of about 1.022, 75

a refractive index at 25° C. of about 1.465, an acid number of 0.15, and a pH in 4% solution of 8.7.

The hydrogenated fish oil and ethylene oxide reaction product were heated to about 65 to 70° C. About 207 grams of triethanolamine were then added to the liquid mixture and the temperature was thereafter increased to about 85° C. to form a clear solution. Sufficient hot water 10 at a temperature between about 75° and 80° C. was then added to the solution to make a 15%, by weight, dispersion. The addition of water was completed within a period of no more than 30 minutes and during the entire period the temperature of the solution was maintained at a minimum of 75° C., the solution being vigorously stirred during the addition of the water. Thereafter, the dispersion was quickly cooled, within a period of about 30 minutes, to a temperature 15 of about 20° C. by means of a cooling coil. The operations of adding water and stirring were conducted so as to prevent the sucking in of air. 1700 grams of tetrachlorphenol, dissolved in 10 liters of water were then added to the 15%, by weight, dispersion.

A dispersion of very fine particle size was obtained. A portion of the 15% dispersion diluted with water to form a 1.5%, by weight, dispersion showed a light transmission of over 80% by the 20 Fischer Electrophotometer A. C. Model. The original 15% solution had a light transmission of 65%.

A 1.5% aqueous dispersion was applied to wet, freshly spun and washed 75 denier, 30 filament, 25 untwisted, continuous-filament, viscose rayon yarn while the yarn was being temporarily stored on a thread-advancing, thread-storing reel, just prior to the drying stage of a continuous rayon spinning and processing machine as described, 30 for example, in Torrence Patent No. 2,284,497. The yarn was there treated for about ten to fifteen seconds. The treated yarn was continuously advanced to a succeeding thread-advancing, thread-storage device upon which it was dried 45 and thereafter collected on bobbins.

Then the yarn was given about 30 to 35 turns per inch twist and thereafter knitted into hosiery. Ether extractions of the hosiery showed a deposit on the yarn of 3 1/4% to 3 1/2%, by weight, 50 of the yarn-conditioning composition. The hosiery was easily and quickly scoured free of its yarn-conditioning composition by washing in aqueous detergent compositions. The hosiery was remarkably free from snags, pulls and filament breakages, had a very uniform construction and was of very desirable quality.

Although the foregoing example illustrates the application of the invention to hosiery type viscose rayon, i. e. regenerated cellulose, yarns as 60 produced by the continuous rayon spinning and processing methods, it is to be understood that the invention is not intended to be limited thereto. The invention may be employed with advantage in producing staple fiber yarns, and 65 yarns of any denier useful in the textile field. The yarn-treating composition of this invention may also be employed with yarns made from nonmetallic, organic filamentary materials such as, for example, cellulose acetate, cotton, nylon, natural and artificial wools, etc. It may be applied to yarns in package form or in skein form as distinguished from the method described in 70 the above example. Such packages or skeins may be immersed with advantage in solutions of the composition ingredients, such as, for example, in

aqueous dispersions, and thereafter the yarn may be fabricated by the usual methods into textile products.

I claim:

1. A yarn which has been treated with a composition comprising hydrogenated fish oil and a product formed by reacting at least about 20 moles of an alkylene oxide with one mole of a partial polyester of a fatty acid containing at least twelve carbon atoms and a polyhydric alcohol selected from the group consisting of hexahydric alcohols and the anhydro derivatives of such alcohols; said hydrogenated fish oil and ester reaction product being present in said composition in proportions, by weight, of about 0.82 to 1 parts of said hydrogenated fish oil to 1 part of said ester reaction product; said hydrogenated fish oil having a melting point of between about 30° C. and 60° C.

2. A yarn which has been treated with a composition comprising a hydrogenated fish oil and a reaction product formed by reacting at least about twenty moles of ethylene oxide with one mole of a sorbitan partial polyester of a fatty acid containing at least twelve carbon atoms; said composition ingredients being present in proportions, by weight, of about 1 part of said ethylene oxide reaction product to from about .82 to 1 parts of the hydrogenated fish oil; said hydrogenated fish oil having a melting point between 30° C. and 60° C. and an iodine number below about 50, and said yarn having been treated so that in a dry state it contains a total of about .75% to 10.0%, by weight, of said composition ingredients.

3. A yarn which has been treated with a composition comprising a hydrogenated fish oil and a reaction product formed by reacting at least about twenty moles of ethylene oxide with one mole of a partial polyester of a fatty acid containing at least twelve carbon atoms and a polyhydric alcohol selected from the group consisting of hexahydric alcohols and the anhydro derivatives of such alcohols; said hydrogenated fish oil and ethylene oxide reaction product being present in proportions, by weight, of about 1 part of said ethylene oxide reaction product to from about .82 to 1 parts of the hydrogenated fish oil; said hydrogenated fish oil having a melting point between 30° C. and 60° C. and an iodine number below about 50 and said yarn having been treated so that in a dry state it contains a total of about .75% to 10.0%, by weight, of said ingredients.

4. A regenerated cellulose yarn which has been treated with composition comprising a hydrogenated fish oil and a reaction product formed by reacting at least about twenty moles of ethylene oxide with one mole of sorbitan trioleate; said hydrogenated fish oil and ethylene oxide reaction product being present in said composition in proportions, by weight, of about 1 part of said ethylene oxide reaction product to from about .82 to 1 parts of the hydrogenated fish oil; said hydrogenated fish oil having a melting point between 40° C. and 55° C. and an iodine number below about 45; said yarn having been treated so that in a dry state it contains a total of about .8% to 4% of said composition ingredients.

5. A regenerated cellulose yarn which has been treated with a composition comprising a hydrogenated fish oil and a reaction product formed by reacting at least about twenty moles of ethylene oxide with one mole of mannnit trioleate; said hydrogenated fish oil and ethylene oxide reaction product being present in proportions, by

weight, of about 1 part of said ethylene oxide reaction product to from about .82 to 1 parts of the hydrogenated fish oil; said hydrogenated fish oil having a melting point between 40° C. and 55° C. and an iodine number below about 45, said yarn having been treated so that in a dry state it contains a total of about .8% to 4%, by weight, of said ingredients.

6. A composition for the treatment of yarns, threads, filaments, and the like, comprising a hydrogenated fish oil and a product formed by reacting at least about 20 moles of an alkylene oxide with one mole of a partial polyester of a fatty acid containing at least twelve carbon atoms and a polyhydric alcohol selected from the group consisting of hexahydric alcohols and the anhydro derivatives of such alcohols; said hydrogenated fish oil and ester reaction product being present in said composition in proportions, by weight, of about 0.82 to 1 parts of said hydrogenated fish oil to 1 part of said ester reaction product; said hydrogenated fish oil having a melting point of between about 30° C. and 60° C.

7. A composition for the treatment of yarns, threads, filaments, and the like, comprising a hydrogenated fish oil and a product formed by reacting at least about twenty moles of ethylene oxide with one mole of a partial polyester of a fatty acid containing at least twelve carbon atoms and a polyhydric alcohol selected from the group consisting of hexahydric alcohols and the anhydro derivatives of such alcohols; said hydrogenated fish oil and ester reaction product being present in said composition in proportions, by weight, of about 0.82 to 1 parts of said hydrogenated fish oil to 1 part of said ester reaction product; said hydrogenated fish oil having a melting point of between about 30° C. and 60° C.

8. A composition for the treatment of yarns, threads, filaments, and the like comprising a hydrogenated fish oil and a product formed by reacting at least about twenty moles of ethylene oxide with one mole of a partial polyester of a fatty acid containing at least twelve carbon atoms and a polyhydric alcohol selected from the group consisting of hexahydric alcohols and the anhydro derivatives of such alcohols; said composition ingredients being present in proportions, by weight, of about 1 part of said ethylene oxide reaction product to from about .82 to 1 parts of the hydrogenated fish oil; said hydrogenated fish oil having a melting point between 30° C. and 60° C. and an iodine number below about 50.

9. A composition for the treatment of yarns, threads, filaments, and the like, comprising an aqueous dispersion of about .3% to 5.0%, by weight, combined concentration of a hydrogenated fish oil and a product formed by reacting at least about twenty moles of ethylene oxide with one mole of a sorbitan partial polyester of a fatty acid containing at least twelve carbon atoms; said composition ingredients being present in proportions, by weight, of about 1 part of said ethylene oxide reaction product to from about .82 to 1 parts of the hydrogenated fish oil; said hydrogenated fish oil having a melting point between 30° C. and 60° C. and an iodine number below about 50.

10. A composition for the treatment of regenerated cellulose yarns, threads, filaments, and the like, comprising an aqueous dispersion of about .3% to 5.0%, by weight, combined concentration of a hydrogenated fish oil and a product formed by reacting at least about twenty moles of ethylene oxide with one mole of sorbitan tri-

oleate; said composition ingredients being present in proportions, by weight, of about 1 part of said ethylene oxide reaction product to from about .82 to 1 parts of the hydrogenated fish oil; said hydrogenated fish oil having a melting point between 40° C. and 55° C. and an iodine number below about 45.

11. A composition for the treatment of regenerated cellulose yarns, threads, filaments, and the like, comprising an aqueous dispersion of about .3% to 5.0%, by weight, combined concentration of a hydrogenated fish oil and a product formed by reacting at least about twenty moles of ethylene oxide with one mole of mannitian trioleate; said composition ingredients being present in proportions, by weight, of about 1 part of said ethylene oxide reaction product to from about .82 to 1 parts of the hydrogenated fish oil; said hydrogenated fish oil having a melting point between 40° C. and 55° C. and an iodine number below about 45.

12. A composition for the treatment of regenerated cellulose yarns, threads, filaments, and the like, comprising an aqueous dispersion of about .3% to 5.0%, by weight, combined concentration of a hydrogenated fish oil and a product formed by reacting at least about twenty moles

of ethylene oxide with one mole of sorbitan tri-laurate; said composition ingredients being present in proportions, by weight, of about 1 part of said ethylene oxide reaction product to from about .82 to 1 parts of the hydrogenated fish oil; said hydrogenated fish oil having a melting point between 40° C. and 55° C. and an iodine number below about 45.

10

ROBERT D. MACLAURIN.

## REFERENCES CITED

The following references are of record in the file of this patent:

## 18 UNITED STATES PATENTS

| Number    | Name              | Date          |
|-----------|-------------------|---------------|
| 2,005,785 | Hibbert           | June 25, 1935 |
| 2,073,630 | Gardthausen       | Mar. 16, 1937 |
| 2,082,278 | Ferguson          | June 1, 1937  |
| 2,133,300 | Linebarger et al. | Oct. 18, 1938 |
| 2,246,735 | Kline et al.      | June 24, 1941 |
| 2,403,305 | Rossiter          | July 2, 1946  |

## OTHER REFERENCES

25 "Spans and Tweens," pamphlet published by Atlas Powder Co., Dec. 1943, pages 2 and 11.